

(No Model.)

W. McCOMBIE.  
JOURNAL BRASS.

No. 433,301.

Patented July 29, 1890.

*Fig. 1.*



*Fig. 2.*



Witnesses:

F. C. Gibson  
C. D. Davis

Inventor:  
William McCombie  
By his Attorney  
C. M. Alexander

# UNITED STATES PATENT OFFICE.

WILLIAM MCCOMBIE, OF CHICAGO, ILLINOIS.

## JOURNAL-BRASS.

SPECIFICATION forming part of Letters Patent No. 433,301, dated July 29, 1890.

Application filed May 2, 1890. Serial No. 350,366. (No model.)

*To all whom it may concern:*

Be it known that I, WILLIAM MCCOMBIE, a citizen of the United States, residing at Chicago, in the county of Cook and State of Illinois, have invented certain new and useful Improvements in Journal-Brasses, of which the following is a specification, reference being had therein to the accompanying drawings.

10 This invention relates to certain improvements in journal-brasses; and it has for its object to provide a journal-brass with an anti-friction bearing having two distinct bearing surfaces of dissimilar metals or alloys possessing different degrees of hardness, the softer metal or alloy projecting beyond the bearing-surface of the harder metal or alloy to receive the first bearing of the journal, the two metals or alloys being of such nature that their contiguous surfaces will be intimately united, cemented, or welded in forming the lining, as more fully hereinafter specified.

In the accompanying drawings, forming part of this specification, Figure 1 represents a longitudinal, and Fig. 2 a sectional, view of a journal-brass, showing my improved bearings applied thereto.

25 In the said drawings, the letter A indicates a shell of the usual construction, and B and C the bearing-blocks forming the lining thereof. The block C is preferably formed of sheet-lead, and the block B of an anti-friction alloy, such as Babbitt metal or other similar compound.

30 In constructing this brass the shell is placed in the mold, as usual, and the sheet of lead C, suitably curved and beveled at its edges, is located in the mold in proper position to leave a suitable space between its inner face and the inner face of the shell A to receive the 35 filling of Babbitt metal or alloy B, which is fused and poured in in the usual manner. The inner face of the lead, or that face opposite the inner face of the shell, previous to being placed in position in the mold, is suitably 40 prepared, so that when the alloy is poured in

it will unite with or become cemented, soldered, or welded to the sheet of lead, so as to form virtually one block having bearing-surfaces of different degrees of hardness. The surface of the lead may be prepared to receive 50 the alloy by coating it with a suitable flux, such as a mixture of rosin and borax. The temperature of fusion of the soft and the harder block must be nearly the same, so that the harder metal will when poured in make 55 only a surface fusion of the softer metal, in order to unite therewith, and not be sufficiently hot to fuse the entire body of the softer metal and destroy its form.

Any two dissimilar metals or alloys may be 60 used for the lining; but, as before stated, I prefer to employ lead in conjunction with a suitable alloy of a melting temperature about that of lead. In practice I have found an alloy composed of the following ingredients, 65 in about the proportions named, to answer well: copper, four pounds; tin, forty pounds; antimony, twenty-six pounds; lead, one hundred and thirty pounds. It is evident, however, that other metals may be employed to 70 produce an alloy having the proper characteristics without departing from the spirit of my invention.

Having thus described my invention, what I claim, and desire to secure by Letters Patent, is—

A journal-bearing consisting of a suitable shell, a block composed of a suitable alloy, and a thin sheet of softer metal seated within said block and projecting beyond its bearing-surface, the block and alloy being cemented together at their contiguous surfaces, substantially as and for the purposes specified.

In testimony whereof I affix my signature in presence of two witnesses.

WILLIAM MCCOMBIE.

Witnesses:

PETER F. BIESEN,  
JAMES MCCOMBIE.